

## UNITED STATES PATENT OFFICE

2,692,194

## NITROPARAFFIN FUEL

John A. Hannum, Detroit, Mich., assignor to  
 Borg-Warner Corporation, Chicago, Ill., a corporation of Illinois

No Drawing. Application June 9, 1949,  
 Serial No. 98,157

4 Claims. (Cl. 52—5)

1

This invention relates to thermally stabilizing various nitro aliphatic materials used as prime mover fuels and more particularly the materials disclosed in copending application Serial No. 687,213 filed July 30, 1946, in the name of John A. Hannum, now Patent No. 2,537,526. This application is a division of application Serial No. 772,220, filed September 4, 1947, in the names of John A Hannum and Joseph N. Epel.

The fuels identified in the copending application referred to above as filed in the name of John A Hannum possess certain valuable properties as prime mover propellants, particularly for airborne devices, although they may also be efficiently used for other prime movers under a variety of circumstances as in aircraft, under-water craft, land vehicles and stationary installations. Furthermore these materials may be used as a source of power for particular types of devices such as rockets, ram-jets and the like.

Under many operating conditions it is desirable to thermally stabilize the fuel, as by providing a catalyst to improve its combustion characteristics. Heretofore certain fuel additives have been used as catalysts to aid the fuel combustion but, unfortunately, they also act as depressants to some extent to lower the normal explosion temperatures of the material, making it less safe to handle and more liable to premature combustion or explosion than it was before addition of the catalyst. So far as is known, such additives have not heretofore been used with this class of materials to raise the threshold without rendering them materially less useful as fuels.

A general object of the present invention is to provide an improved fuel of this kind. Another object is to provide an additive for use with fuels, particularly nitro aliphatic fuels, by which their tendency to explode prematurely in consequence of the addition of the catalyst is decreased and the safety with which they may be handled improved. Still another object is to provide an additive that acts as a catalyst to a fuel to improve its operating characteristics as by enabling it to burn continuously rather than intermittently. Other objects of the invention will become apparent from the specification, it being understood that certain departures may be made from the following description without departing from the scope of the invention which is limited solely by the attached claims.

As indicated above, the present invention is adapted for use with the fuels that are disclosed in the copending application and that are in the

2

form of liquid nitro aliphatic hydrocarbons, the terms nitro aliphatic and nitroparaffin as hereinafter used being construed herein to include both mono and polynitro derivatives. Such fuels are limited to those that contain not more than one nitro group for each carbon atom present. A preferred form of such fuel is nitromethane,  $\text{CH}_3(\text{NO}_2)$ , that itself contains much of the oxygen required during the combustion of the fuel elements in it. It is contemplated that other fuels from the class of nitro aliphatic liquids may be used in the present invention.

Examples of such fuels, in addition to nitromethane, are:

|    |                       |                                                               |
|----|-----------------------|---------------------------------------------------------------|
| 15 | Nitroethane           | $\text{CH}_3\text{CH}_2\text{NO}_2$                           |
|    | 1-nitropropane        | $\text{CH}_3\text{CH}_2\text{CH}_2\text{NO}_2$                |
| 20 | 2-nitropropane        | $(\text{CH}_3)_2\text{CH}.\text{NO}_2$                        |
|    | 1,1-dinitropropane    | $\text{C}_2\text{H}_5.\text{CH}(\text{NO}_2)_2$               |
|    | 2,2-dinitropropane    | $(\text{CH}_3)_2\text{C}(\text{NO}_2)_2$                      |
| 25 | 1,2-dinitropropane    | $\text{CH}_2\text{NO}_2.\text{CHNO}_2.\text{CH}_3$            |
|    | 1,3-dinitropropane    | $\text{CH}_2\text{NO}_2.\text{CH}_2.\text{CH}_2\text{NO}_2$   |
|    | 1,1-dinitroethane     |                                                               |
| 30 |                       | $\text{CH}_3.\text{CH}(\text{NO}_2)_2$                        |
|    | 1,2,3-trinitropropane | $\text{CH}_2\text{NO}_2.\text{CHNO}_2.\text{CH}_2\text{NO}_2$ |
|    | 1,1,1-trinitropropane | $\text{C}(\text{NO}_2)_3.\text{CH}_2\text{CH}_3$              |

35 Such nitro aliphatics included as fuels within the scope of this invention include mononitromethane, dinitroethane and trinitropropane and those nitroethanes and nitropropanes below them in oxygen content but no nitroethanes or nitropropanes that are higher in oxygen content, as for instance dinitromethane. These are all to be distinguished from aromatic fuels such as the nitrobenzols that are dangerous to handle even by skilled persons to say nothing of persons who are not skilled in this art.

40 An advantage of using nitromethane or a similar partially nitrated aliphatic hydrocarbon as listed above resides in the fact that it contains a considerable proportion of the oxygen that is required during combustion to burn the carbon or hydrogen in the fuel. This in turn does not require the presence of as much air or other oxidizing agent as would otherwise be necessary. 45 These fuel components are non-brisant nitro

aliphatic compounds, non-brisant within the terms of this disclosure meaning that the fuel may be burned in contact with chilled iron without producing the Munroe effect.

Although such fuels are non-brisant as defined above it frequently is desirable to modify their explosion characteristics. When pure nitromethane is heated, it has a threshold explosion temperature of 593.6° Fahrenheit. As indicated above, the addition of certain materials serves to depress to some extent the normal explosion temperatures of pure nitromethane. Insofar as is known no additive has been available until the present invention that modifies the explosion characteristics of nitromethane by suppressing its tendency to explode at or even below its normal explosion temperatures and still preserves and improves the desirable properties of nitromethane as a fuel.

The addition of a small amount, from a trace to substantially two percent by weight of the total fuel mixture, of a chemical compound which may be defined as including an atom of an element with predominantly metallic properties ("Metalloid"), a plurality of oxygen atoms, and a poly-substituted amine radical both improves the combustion qualities of the fuels outlined above and modifies their explosion characteristics in the respects mentioned. A material that acts to raise the threshold explosion temperature of the fuels listed above is the tertiary amine, pyridine salt of uranyl acetylacetone  $\text{UO}_2(\text{C}_5\text{H}_7\text{O}_2)_3\text{H}\cdot\text{C}_5\text{H}_5\text{N}$ . As an example of the utility of the herein described invention, it is pointed out that when approximately 1% by weight of the pyridine salt of uranyl acetylacetone is added to nitromethane, there is found to be an accompanying suppression of the tendency to explode at temperatures below 615.1° Fahrenheit, an increase of approximately 20 degrees over the threshold explosion temperature.

It is important that such salts be relatively stable in the fuels to which they are added and

do not readily break down except incident to the process of combustion.

A fuel mixture made up in accord with the present invention will include one or more of the fuels listed above to make up more than 98 percent but less than 100 percent by weight of the whole. From two percent to a trace by weight will be made up of one or more stabilizers of the kind described herein. These materials will act in varying degrees to stabilize the various nitro aliphatic fuels listed above, which they do by modifying their explosion characteristics; furthermore, inasmuch as they break down incident to the process of combustion of the fuel to yield finely divided metallic oxides, they act as catalysts, causing the fuel to burn steadily and quietly, as distinguished from intermittently, in the combustion zone.

It is intended that the patent shall cover, by suitable expression in the appended claims, whatever features of patentable novelty reside in the invention.

I claim:

1. A fuel mixture comprising a nitroparaffin and from a trace to two percent by weight of the pyridine salt of uranyl acetylacetone.
2. A fuel mixture comprising nitromethane and the pyridine salt of uranyl acetylacetone, the quantity of the latter being a minor fraction of the total of the ingredients making up the mixture.
3. A fuel mixture comprising a nitromethane and from a trace to two percent by weight of the pyridine salt of uranyl acetylacetone.
4. A fuel mixture comprising a liquid nitroparaffin containing not more than one nitro group for each carbon atom present and the pyridine salt of uranyl acetylacetone, the quantity of the latter being a minor fraction of the total of the ingredients making up the mixture.

No references cited.